# EUROPEAN PATENT SPECIFICATION

(11) **EP 0 765 012 B1**
(45) Date of publication and mention of the grant of the patent: **07.07.1999**
(21) Application number: 95942805.3
(22) Date of filing: 21.12.1995
(51) Int. Cl.: H01J 7/18

(54) **NON-VAPORISING GETTER AND METHOD OF OBTAINING THE SAME**
NICHTVERDAMPFBARES GETTERMATERIAL UND VERFAHREN ZU SEINER HERSTELLUNG
DEGAZEUR NON VOLATILE ET SON PROCEDE D'OBTENTION

(30) Priority: 29.12.1994 RU 94045576
(43) Date of publication of application: 26.03.1997
(73) Proprietor: TOVARISCHESTVO S OGRANICHENNOI OTVETSTVENNOSTJU "TEKHNOVAK + ", Moscow, 123479 (RU)
(72) Inventor: REUTOVA, Nina Pavlovna, Moscow, 107014 (RU); MANEGIN, Sergei Jurievich, Moscow, 109241 (RU); PUSTOVOIT, Jury Mikhailovich, Moscow, 123060 (RU); STOLYAROV, Vladimir Leonidovich, Moscow, 123479 (RU)
(74) Representative: Adorno, Silvano
(86) International application number: RU9500276
(87) International publication number: WO9621958

(56) References cited:
- DE-A- 3 031 471
- FR-A- 2 370 101
- GB-A- 1 548 581
- GB-A- 2 161 182
- DATABASE WPI Week 8715 Derwent Publications Ltd., London, GB; AN 87-106498 XP002025296 & SU 1 120 867 A (DAVYDENKO) , 7 September 1986
- DATABASE WPI Week 9304 Derwent Publications Ltd., London, GB; AN 93-034073 XP002025297 & SU 1 715 496 A (ATOM ENERGY INST) , 29 February 1992

## Description

### FIELD OF TECHNOLOGY

The present invention relates to vacuum techniques, specifically to nonevaporable getter and a process for its production.

The invention may be used as a pump for creating and maintaining high vacuum in electronic vacuum devices, e.g. in a cathode-ray tube, in an optical converter, gyroscope, etc., in elementary particles sources and accelerators, e.g. in a thermonuclear plant of TOKAMAK T-15 type.

Preferably the present invention may be used for creating vacuum in devices reducing heat transfer from environment to thermostated media, e.g. in a vacuum flasks, a liquified gas storage, in pipelines for gas and crude oil transportation from wells, which pipelines are thermally insulated to protect environment in the permafrost zone.

Also the present invention may be successfully used for inert gases purification.

### PRIOR ART

Presently intensive development of novel technologies in. e.g. semiconductors production and use, sets stringent requirements to stability of n-type and p-type conduction in p-n-junctions, which conduction is disturbed by detrimental gaseous impurities (i.e. O₂, CO, CO₂, H₂O, N₂ etc.) present in the zone of the treatment of such semiconductors.

Said detrimental impurities are removed by pumping them out from the treatment zone using sorption pumps based on nonevaporable getters, the decrease in the concentration level of detrimental gaseous impurities in said zone depending on the their sorption rate. Therefore the development of getters having improved sorption rate is a matter of great importance. An attempt was made to produce a getter having increased sorption rate (the USSR Inventor's Certificate No. 1715496). The known getter has three layers, one of which being a supporting layer, is made of a plastic material selected from a group comprising, e.g. Fe, Ni or their alloys, and two other surface getter layers each are made of a zirconium-based material, containing, e.g. 16 % by weight of aluminium, the balance being zirconium, or 30 % by weight of vanadium, 20 % by weight of titanium, the balance being zirconium.

Known is the process for producing a getter based on zirconium, comprising the following operations:
- simultaneous feeding into a deformation zone a powder material forming a supporting layer and selected from, e.g. a group comprising Fe, Ni or the alloys thereof, and a zirconium-based powder material comprising 16 % by weight of aluminium (Al), the balance being zirconium (Zr), or 30 % by weight of vanadium (V), 20 % by weight of titanium (Ti), the balance being zirconium (Zr), and forming getter layer, zirconium-based materials being fed to the both sides of the material forming the supporting layer. In said deformation zone said powder materials are formed by rolling, as a result of which a getter blank in the form of a three-layer ribbon is produced. When said ribbon is leaving the deformation zone it is cut into standard sections, e.g. 200 mm. Said standard sections of getter blanks are brought into a heating zone wherein vacuum conditions are created and maintained, and heated up to 950-1.000 Celsius degrees. As a result of this the blank material gets sintered and the final getter is produced in the form of a product having improved mechanical properties, namely, increased tensile strength of getter material, e.g. from 6.3 to 6.8 kg/mm², and increased sorption rate, e.g. reaching 1.9 m³/m² s at room temperature, when sorbed hydrogen quantity is 1.3 m³. Pa/kg, after getter activation at 900 Celsius degrees.

In spite of increased tensile strength the known getter shows low mechanical strength of the getter layer because getter layers are made of a material based on a Zr-Al or Zr-V-Ti alloy comprising large amount of intermetallic compounds characterized by increased hardness and brittleness. Therefore when such getters are used under alternating loads, they fail, most often as a result of crumbling. Moreover zirconium-based getter containing 16 % by weight of aluminium causes increased power consumption because high temperature (about 900 Celsius degrees) is required to activate such getter.

Furthermore the known getter has low sorptive capacity with respect to such gases as H₂, O₂, CO₂, CO , N₂, etc. because the supporting layer made of, e.g. Fe, Ni and their alloys, is neutral to gas sorption, and because of low porosity of getter layers being about 20%.

The above process for producing nonevaporable getter is hard to realize because it is difficult to reach an optimal correlation between the thickness of the supporting layer and the total thickness of the getter layer; also said process involves high loss in powder material resulting in increased getter costs.

Moreover known is a nonevaporable getter having increased mechanical strength and improved sorption rate (the SU Patent No. 1750256). The known getter contains from 20 to 35 % by weight of vanadium (V), from 0.1 to 0.5 % by weight of calcium (Ca), and the balance being titanium (Ti).

Said getter shows increased mechanical strength when used under alternating loads, due to high plasticity of the material being a solid solution of vanadium in titanium. The presence of elementary calcium in the getter material contributes to an increased rate of gas sorption because calcium showing high chemical activity to oxygen forms calcium oxide (CaO), and calcium oxide particles being uniformly distributed among metal particles, act as antisintering agent contributing to high porosity of the getter.

The above getter is produced as follows.
Metal powder containing from 20 to 35 % by weight of vanadium, from 0.1 to 0.5 % by weight of calcium, the balance being titanium, is fed into a deformation zone, wherein said powder material is formed by rolling to produce a getter blank in the form of a ribbon. When said ribbon is leaving the deformation zone, it is cut into standard sections, said sections being transported into a heating zone.

In said heating zone a pressure of lower than 1 Pa is created and maintained, and the blank is heated to a temperature lower than 0.6 times the melting point of titanium-vanadium alloy, e.g. to 850 Celsius degrees, with further holding. The getter thus produced is a plate having 22% porosity, sorption rate with respect to hydrogen being 1.8 m³/m²s at room temperature, when the quantity of sorbed hydrogen is 1.3 m³ Pa/kg. Said getter is activated at 300-350 Celsius degrees.

In view of the foregoing a getter having said composition, may be referred to the getters with low activation temperature, which fact allows to develop pumping means requiring low power consumption. Nevertheless due to reduced sorption rate such getter has restricted applicability, e.g. it cannot be used as a stage in a multistage pumping device used in semiconductors production.

### DESCRIPTION OF THE INVENTION

The object of the present invention is to develop a nonevaporable getter having sorptive rate with respect to hydrogen of over 2 m³/m²s at room temperature when the quantity of sorbed hydrogen being 1.3 m³Pa/kg, due to a larger surface contacting the gas to be pumped out.

The object of the invention is achieved by that nonevaporable getter containing from 20 to 35 % by weight of vanadium, from 0.1 to 0.5 % by weight of calcium and the balance being titanium, according to the invention, has porosity from 25 to 65 % by volume.

Said getter has larger number of pores opening at its surface. As a result larger surface contacts the gas to be pumped out, resulting in increased gas sorption rate, e.g. the sorption rate for hydrogen is dver 2 m³/m²·s at room temperature when the quantity of sorbed hydrogen is 1.3 m³ Pa/kg. A getter having the porosity less than 25%, shows hydrogen sorption rate less than 2 m³/m²·s, due to which fact its applicability is restricted. A getter having porosity less than 25% cannot be used, e.g. as a stage in a multistage pumping device used in semiconductors production.

A getter having porosity over 65% has lower mechanical strength, which may result in its crumbling and failing under alternating loads. Such getter cannot be used e.g. in night-vision devices, gyroscopes, etc.

Thus the getter according to the present invention has increased sorption rate (1.5-3 times) after activation at 300-350 Celsius degrees, due to greater open porosity accounted for increased total porosity of the getter.

Also the object of the invention is to develop a process for producing a nonevaporable getter comprising using powder material with branched particles to form porosity in the range from 25 to 65 % in said material.

Said object is achieved by that in the process for producing a nonevaporable getter comprising feeding a metal powder containing from 20 to 35 % by weight of vanadium, from 0.1 to 0.5 % by weight of calcium, the balance being titanium, into a deformation zone wherein said powder material is formed by rolling to produce a getter blank in the form of a ribbon, said ribbon, when leaving the deformation zone, being cut into standard sections, said sections being transported into a heating zone, in said heating zone a pressure of lower than 1 Pa being created and maintained, and the blank being heated to a temperature lower than 0.6 times the melting point of titanium-vanadium alloy, with further holding, producing a getter having the porosity from 22% to 65% by volume, according to the invention, said metal powder has bulk density in the range from about 0.7 to about 1.5 g/cm³, and has less than 70 % by weight of particles having a particle size of less than 50 µm.

Bulk density of a metal powder determines pores quantity and size in formed blank. It is generally known that with less values of bulk density the greater values of porosity of the final product are obtained, and vice versa.

Experiments have shown that when bulk density of the metal powder containing from 20 to 35 % by weight of vanadium, from 0.1 to 0.5 % by weight of calcium, the balance being titanium, is approaching the value of 0.7 g/cm³ , then resulting getter has porosity about 65%, while when bulk density of the above powder is about 1.5 g/cm³, then the resulting getter has porosity about 25%.

The metal powder fed into the deformation zone, should contain less than 70 % by weight of fraction having particle size of less than 50 µm. Then the metal powder will have bulk density about 1.5 g/cm³. In case above metal powder contains less than 20 % by weight of a fraction having particle size of less than 50 µm, bulk density of said powder will be about 0.7 g/cm³.

Preferably getter blank should be heated within the range from about 750 to about 950 Celsius degrees. Said temperature range is determined by the maximum permissible shrinkage level with which the mechanical strength of resulting getter as well as its porosity (25-65 %) are maintained. In case said blank is heated up to less than 750 Celsius degrees in the heating zone, then weaker bonds are formed among the particles, due to low diffusive mobility of metal atoms, which results in reduced mechanical strength of the getter. In case said blank is heated up to over 950 Celsius degrees, considerable shrinkage occurs which causes reduced porosity of the getter thus resulting in lower sorption rate.

When the porosity of a getter blank is less than 45%, a standard section of said blank may be coiled.

Known is the fact that a ribbon-type blank shows low mechanical strength, which strength reduces when porosity increases. Experiments have shown that when getter blank having porosity over 45% is coiled, said blank fails.

Other objects and advantages of the inventions will be clarified by the following examples of specific embodiments of the present invention.

### VARIANTS OF SPECIFIC EMBODIMENTS OF THE INVENTION

A nonevaporable getter according to the invention containing from 20 to 35 % by weight of vanadium, from 0.1 to 0.5 % by weight of calcium, the balance being titanium, has porosity from about 25% to about 65% (by volume).

The getter according to the invention has hydrogen sorption rate over 2 m³/m²·s at room temperature, when the quantity of sorbed hydrogen is 1.3 m³Pa/kg, the getter being activated at from 300 to 350 Celsius degrees.

Said properties allow to use said getter in sorption pumps used in elementary particles sources and accelerators, e.g. in thermonuclear plants wherein high pumping rate is to be provided in restricted spaces.

To produce a getter having abovementioned properties a process is provided according to the invention, said process comprising the following operations:

Metal powder containing from 20 to 35 % by weight of vanadium, from 0.1 to 0.5 % by weight of calcium, the balance being titanium, and having bulk density within the range from about 0.7 to about 1.5 g/cm³ is fed into a deformation zone. Said metal powder contains less than 70% (by weight) of fraction having particle size of less than 50 µm. Within said deformation zone a force is exerted, e.g. 1 t/cm² , exceeding compression strength of said metal powder, which causes plastic deformation of metal particles.

Further metal powder is rolled to form a ribbon blank having uniform density and higher porosity than the porosity of the final product. Ribbon length is much longer than its width, the ribbon having small ; thickness and strength sufficient to transport said ribbon into a heating zone. As a result of rolling a ribbon is produced having the width of, e.g. from 15 to 80 mm, and the thickness of, e.g. from 0.4 to 0.8 mm.

During rolling said metal powder undergoes continuous forming, the volume of the powder reducing because the density of particles placement in said powder increases, though the weight remains constant.

When a getter blank is leaving the deformation zone, it is cut into standard sections which sections, e.g. having the length 200, 70 mm, etc., are transported into a heating zone. In said heating zone the pressure below 1 Pa is created and maintained, under which the partial pressure of chemically active gases (excluding hydrogen) should be below 1.10⁻² Pa in said heating zone, and said getter blank is heated to a temperature lower than 0.6 times the melting point of titanium-vanadium alloy, followed by holding. Said heating temperature is maintained in the range from about 750 to about 950 Celsius degrees. Said temperature range is determined by maximum permissible shrinkage level at which mechanical strength of resulting getter is maintained, namely, tensile strength reaches, e.g. from 1 to 6 kg/mm², and the desired porosity is from 25 to 65 %.

In one variant of specific embodiments of the invention a standard section of said getter blank is coiled, provided that getter porosity is below 45%. It is known that a ribbon-type blank shows low mechanical strength, which strength decreases when the porosity increases. Experiments have shown that when a blank having porosity over 45% is coiled, said blank fails.

### Example 1.

Metal powder containing 28.45 % by weight of vanadium, 0.31 % by weight of calcium, 71.24 % by weight of titanium, having bulk density γ=1.17 g/cm³ is fed into deformation zone, said metal powder containing 57% (by weight) of fraction (q) having particle size of less than 50 µm. Within said deformation zone metal powder is formed by rolling using rollers having the diameter, e.g. ⌀ 100 mm and rolling speed (V) 1.5 m/min. As a result a getter blank of uniform density is produced in the form of a ribbon having thickness (h) of 0.5 mm and width of 30 mm, the porosity of said blank being greater than the porosity of the final product. During rolling said metal powder is continuously formed. After leaving said deformation zone said ribbon-type getter blank is cut into standard sections having length 200 mm, and then said sections are transported into the heating zone. Within said heating zone the pressure of 0.025 Pa is created and maintained, and the blank is heated to the temperature (T) of 850 Celsius degrees, followed by holding during 1 hour. After cooling the blank is removed. Porosity (P) of the final product is 43%, and its tensile strength is 2.1 kg/mm².

Resulting getter has sorption rate (S) with respect to hydrogen of 4.0 m³/m².s at sorption temperature (t) 20 Celsius degrees when the quantity of sorbed hydrogen (Q) is 1.3 m³Pa/kg after getter activation at the temperature (Ta_{KT}) of 350 Celsius degrees during 15 min.

### Example 2.

Metal powder containing 27.20 % by weight of vanadium, 0.21 % by weight of calcium, 72.61 % by weight of titanium, having bulk density γ 0.98 g/cm³ is fed into a deformation zone, said metal powder containing 48% (by weight) of fraction (q) having particle size of less than 50 µm. Within said deformation zone metal powder is formed by rolling using rollers as described in Example 1. As a result a getter blank of uniform density is produced in the form of a ribbon having thickness (h) of 0.5 mm and width of 30 mm, the porosity of said blank being greater than the porosity of the final product. After leaving said deformation zone said ribbon-type getter blank is cut into standard sections. Said standard sections of getter blank having the porosity (P) below 45% are then coiled into coils with 80 mm inner diameter. The length of said standard section is 2.96 m. Coiled getter blank is transported into the heating zone wherein the pressure of 0.025 Pa is created and maintained, and the blank is heated to the temperature (T) of 850 Celsius degrees, followed by holding during 1 hour. After cooling the coiled blank is removed. Resulting getter is characterized by large sorptive surface which is larger than that of the getter as per Example 1. Porosity (P) of the coiled getter is 38.5%, its sorption rate (S) with respect to hydrogen being 3.3 m³/m².s at sorption temperature (t) being 20 Celsius degrees, when the quantity (Q) of sorbed hydrogen is 1.3 m³Pa/kg after getter activation at the temperature (Ta_{KT}) of 350 Celsius degrees during 15 min.

The results of the experiments carried out using metal powder with different bulk densities and applying different sintering temperatures, are provided in the Table.

**TABLE**

| No. | Element content (% by weight) | | | | | | | | |
|---|---|---|---|---|---|---|---|---|---|
| | V | Ca | Ti | γ (g/cm³) | q (%) | T (°C) | P (%) | h mm | S (m³/m²s at t=20°C Q=1.3m³Pa/kg Ta_{KT}=350°C 15 min. |
| 1 | 28.45 | 0.31 | Balance | 1.17 | 57 | 850 | 43 | 0.5 | 4.0 |
| 2 | 27.20 | 0.21 | - " - | 0.98 | 48 | 850 | 38.5 | 0.5 | 3.3 |
| 3 | 27.20 | 0.21 | - " - | 1.46 | 68 | 780 | 32 | 0.65 | 2.9 |
| 4 | 27.20 | 0.21 | - " - | 0.8 | 26 | 900 | 52 | 0.71 | 5.2 |
| 5 | 32.2 | 0.18 | - " - | 0.77 | 18 | 860 | 54 | 0.68 | 7.3 |

wherein
- γ: is bulk density of metal powder;
- q: is the quantity of the fraction having particle sizes less than 50 µm;
- T: is heating temperature;
- P: is getter porosity;
- h: is getter thickness;
- S: is hydrogen sorption rate;
- t: is sorption temperature;
- Q: is the quantity of sorbed hydrogen;
- Ta_{KT}: is getter activation temperature.

### INDUSTRIAL APPLICABILITY

Getter according to the invention having porosity of 30%, when used as the first stage formed by forty plates having dimensions 180x30x0.8 mm in a multistage magnetic discharge pump mounted in accelerator used in semiconductors production, has pumping rate with respect to hydrogen from 0.3 to 2 m³/s.

## Claims

1. A nonevaporable getter containing from 20 to 35 % by weight of vanadium, from 0.1 to 0.5 % by weight of calcium, the balance being titanium, characterized by that said getter has porosity from 25 to 65 % by volume.

2. A process for producing nonevaporable getter comprising the following operations:
feeding metal powder containing from 20 to 35 % by weight of vanadium, from 0.1 to 0.5 % by weight of calcium, the balance being titanium, into a deformation zone, wherein said metal powder being formed by rolling. as a result a getter blank being produced in the form a ribbon, said ribbon after leaving said deformation zone being cut into standard sections, said sections being further transported into a heating zone, in said heating zone the pressure below 1 Pa being created and maintained, and
heating said getter blank to a temperature lower than 0.6 times the melting point of titanium-vanadium alloy, followed by holding, as a result a getter being produced having porosity from 25 to 65 % by volume, characterized by that said metal powder being fed into said deformation zone, has bulk density in the range from about 0.7 to about 1.5 g/cm³, and has less than 70 % by weight of particles having a particle size of less than 50 µm.

3. A process according to Claim 2, characterized by that said getter blank is heated to a temperature within the range from about 750 Celsius degrees to about 950 Celsius degrees.

4. A process according to any of Claims 2-3, characterized by that when the porosity of said getter blank is below 45%, said standard section is coiled.

## Patentansprüche

1. Nichtverdampfbarer Getter, der 20 bis 35 Gew.% Vanadium, 0,1 bis 0,5 Gew.% Kalzium und den Rest Titan enthält, dadurch gekennzeichnet, daß der Getter eine Porosität von 25 bis 65 Vol.% aufweist.

2. Verfahren zur Herstellung eines nichtverdampfbaren Getters, welches die folgenden Arbeitsschritte umfaßt:
Zuführen eines Metallpulvers, das 20 bis 35 Gew.% Vanadium, 0,1 bis 0,5 Gew.% Kalzium und den Rest Titan enthält, in eine Verformungszone, in welcher das Metallpulver durch Walzen geformt wird, wodurch ein Getterrohling in Form eines Bandes erzeugt wird, wobei das Band nach dem Verlassen der Verformungszone in Standardteilstücke geschnitten wird, wobei die Standardteilstücke weiter in eine Erwärmungszone befördert werden, in dieser Erwärmungszone ein Druck von weniger als 1 Pa erzeugt und aufrechterhalten wird, und der Getterrohling auf eine Temperatur erwärmt wird, die geringer als das 0,6-fache des Schmelzpunktes der Titan-Vanadium-Legierung ist, und weiter bei dieser gehalten wird, wodurch ein Getter mit einer Porosität von 25 bis 65 Vol.% erzeugt wird, dadurch gekennzeichnet, daß das Metallpulver, das in die Verformungszone geleitet wird, eine Schüttdichte im Bereich von etwa 0,7 bis etwa 1,5 g/cm³ aufweist und weniger als 70 Gew.% Partikel mit einer Partikelgröße von weniger als 50 µm aufweist.

3. Verfahren nach Anspruch 2, dadurch gekennzeichnet, daß der Getterrohling auf eine Temperatur im Bereich von etwa 750 Grad Celsius bis etwa 950 Grad Celsius erwärmt wird.

4. Verfahren nach einem der Ansprüche 2 und 3, dadurch gekennzeichnet, daß das Standardteilstück aufgerollt wird, wenn die Porosität des Getterrohlings unter 45 % liegt.

## Revendications

1. Un dégazeur non volatile contenant de 20 à 35 % en poids de vanadium, de 0,1 à 0,5 % en poids de calcium, le reste étant du titane, caractérisé en ce que ledit dégazeur a une porosité de 25 à 65 % en volume.

2. Un procédé de réalisation d'un dégazeur non volatile comprenant les opérations suivantes :
amener une poudre métallique contenant de 20 à 35 % en poids de vanadium, de 0,1 à 0,5 % en poids de calcium, le reste étant du titane, dans une zone de formage, où ladite poudre métallique est mise en forme par laminage, à la suite de quoi est obtenu un flan de dégazeur sous la forme d'un ruban, ledit ruban après avoir quitté ladite zone de formage étant coupée en sections standard, lesdites sections étant en outre transportées dans une zone de chauffage, zone de chauffage dans laquelle est créée et maintenue une pression inférieure à 1 Pa, et chauffer ledit flan de dégazeur à une température inférieure à 0,6 fois le point de fusion de l'alliage titane-vanadium, suivi par un maintien, à la suite de quoi est réalisé un dégazeur présentant une porosité de 25 à 65 % en volume, caractérisé en ce que ladite poudre métallique qui est amenée dans ladite zone de formage a une densité en vrac dans la gamme d'environ 0,7 à environ 1,5 g/cm³, et présente moins de 70 % en poids de particules ayant une granulométrie inférieure à 50 µm.

3. Un procédé selon la revendication 2, caractérisé en ce que ledit flan de dégazeur est chauffé à une température à l'intérieur de la gamme d'environ 750° Celsius à environ 950° Celsius.

4. Un procédé selon une quelconque des revendications 2-3, caractérisé en ce que, lorsque la porosité dudit flan de dégazeur est en dessous de 45 %, ladite section standard est bobinée.
